



US006290337B1

(12) **United States Patent**  
Radke

(10) **Patent No.:** US 6,290,337 B1  
(45) **Date of Patent:** Sep. 18, 2001

(54) **PRINT HEAD FOR INK-JET PRINTING AND A METHOD FOR MAKING PRINT HEADS**

(75) Inventor: **Garold E. Radke**, Lebanon, OR (US)

(73) Assignee: **Hewlett-Packard Company**, Palo Alto, CA (US)

(\*) Notice: Subject to any disclaimer, the term of this patent is extended or adjusted under 35 U.S.C. 154(b) by 0 days.

(21) Appl. No.: **09/149,766**

(22) Filed: **Sep. 8, 1998**

**Related U.S. Application Data**

(63) Continuation-in-part of application No. 08/742,118, filed on Oct. 31, 1996.

(51) **Int. Cl.<sup>7</sup>** ..... **B41J 2/05**

(52) **U.S. Cl.** ..... **347/65**; 347/45; 347/47; 347/44

(58) **Field of Search** ..... 347/45, 47, 65, 347/44; 156/319

(56) **References Cited**

**U.S. PATENT DOCUMENTS**

- 4,077,932 \* 3/1978 Columbus ..... 260/29.6  
4,101,356 7/1978 Savelkouls .  
4,535,343 8/1985 Wright et al. ..... 346/140 R  
4,623,906 \* 11/1986 Chandrashekhar et al. ..... 347/47  
4,922,607 5/1990 Doan et al. .

|             |        |                                   |
|-------------|--------|-----------------------------------|
| 4,953,287   | 9/1990 | West et al. .                     |
| 5,086,307   | 2/1992 | Noguchi et al. ..... 346/140 R    |
| 5,275,695 * | 1/1994 | Chang et al. ..... 216/27         |
| 5,493,302   | 2/1996 | Sandbach, Jr. et al. ..... 347/47 |
| 5,493,320 * | 2/1996 | Sandbach, Jr. et al. ..... 347/47 |
| 5,807,430   | 9/1998 | Zheng et al. .                    |
| 5,807,922 * | 9/1998 | Thames et al. ..... 524/725       |
| 6,054,011   | 4/2000 | Radke et al. .                    |

\* cited by examiner

*Primary Examiner*—John Barlow

*Assistant Examiner*—M Shah

(57) **ABSTRACT**

A print head for ink-jet printing including an orifice plate with an intermediate layer of reinforcement material bonded thereto, an ink barrier layer, and an adhesion promoter located between the intermediate layer and the barrier layer. The adhesion promoter bonds the intermediate layer to the barrier layer. Exemplary adhesion promoters include organosilane compositions, polyacrylic acid, polymethylacrylic acid, and mixtures thereof. Representative intermediate layers include oxidizable metals (e.g. chromium, tantalum, and mixtures thereof) and silicon-containing compositions (e.g. silicon dioxide, silicon nitride, silicon carbide, and mixtures thereof). In a process for making a print head, an adhesion promoter is applied to the orifice plate/intermediate layer combination which is thereafter bonded to the barrier layer using the adhesion promoter. All of these components are secured together through the application of pressure and heat.

**10 Claims, 3 Drawing Sheets**





Fig. 1



Fig. 2



Fig. 3



Fig. 4



Fig. 5



Fig. 6

## PRINT HEAD FOR INK-JET PRINTING AND A METHOD FOR MAKING PRINT HEADS

### CROSS-REFERENCE TO RELATED APPLICATION

This application is a continuation-in-part of co-pending U.S. patent application Ser. Ser. No. 08/742,118 filed Oct. 31, 1996 which is incorporated herein by reference for all that it discloses.

### FIELD OF INVENTION

The present invention generally relates to ink-jet printing and, more particularly, to print heads for ink-jet print cartridges and methods for manufacturing such print heads.

### BACKGROUND OF THE INVENTION

The art of ink-jet technology is relatively well developed. Commercial products such as computer printers, graphics plotters, and facsimile machines employ ink-jet technology for producing printed media. Hewlett-Packard's contributions to this technology are described, for example, in various articles in the *Hewlett-Packard Journal*, Vol. 36, No. 5 (May 1985), Vol. 39, No. 4 (August 1988), Vol. 39, No. 5 (October 1988), Vol. 43, No. 4 (August 1992), Vol. 43, No. 6 (December 1992), and Vol. 45, No. 1 (February 1994).

Generally, an ink-jet image is formed when a precise pattern of dots is ejected from drop generating device known as a "print head" onto a printing medium. The typical ink-jet print head has an array of precisely formed nozzles in an orifice plate that is attached to an ink barrier layer on a thermal ink-jet print head substrate. The substrate incorporates an array of firing chambers that receive liquid ink (colorant dissolved or dispersed in a solvent) from an ink reservoir. Each chamber has a thin-film resistor, known as a "firing resistor", located opposite each nozzle so ink can collect between the firing resistor and the nozzle. When electric printing pulses heat the thermal ink-jet firing resistor, a small volume of ink adjacent the firing resistor is heated, vaporizing a bubble of ink, and thereby ejecting a drop of ink from the print head. The droplets strike the printing medium and then dry to form "dots" that, when viewed together, form the printed image.

The physical arrangement of orifice plate, ink barrier layer, print head substrate, and various intermediate layers on the substrate is further described and illustrated at page 44 of the *Hewlett-Packard Journal* of February 1994, cited above.

In ink-jet print head technology, the orifice plate is expected to be permanently attached to the ink barrier layer on the print head substrate. Delamination of the interface between the orifice plate and the barrier layer has always been a problem but recently the problem has increased in significance.

Delamination principally occurs from environmental moisture and the ink itself. Environmental moisture develops from storing the print cartridge in a capping station on the printer, in normal, open room storage, or in shipping packages. Environmental moisture has become an increasing problem because print cartridges are increasingly being subjected to longer and longer periods of storage. As for ink, it has become a problem because some inks wick much more into the interface between the orifice plate and the barrier. Such inks contain surfactants and solvents that increase the capillary effect at the orifice plate-ink barrier interface.

Delamination of the orifice plate is manifested in several ways. Full delamination occurs when the orifice plate falls

off the print cartridge. The print cartridge deprimes, and the electrical leads within the printer can be shorted out. When partial delamination occurs, print cartridge performance and print quality can degrade markedly. Delamination changes the architecture of the ink conduits and firing chambers. Fluidic isolation of the firing chambers can be lost, cross-talk between the firing chambers and ink conduits can develop, and if there are inks of different colors in adjacent chambers, color mixing can occur.

U.S. Pat. No. 5,493,320 entitled "Ink-jet Printing Nozzle Array Bonded to a Polymer Ink Barrier Layer" by Sandbach et al. issued on Feb. 20, 1996 recognizes the problem of orifice plate-ink barrier layer delamination. This patent, however, does not go far enough and does not contemplate the measures needed to be taken against very aggressive inks and increased storage times in printers, open room environment, or shipping packages.

It will be apparent from the foregoing that although there are many varieties of print cartridges and processes for making them, there is still a need for an approach that avoids both full and partial delamination of the orifice plate-ink barrier layer interface.

### SUMMARY OF THE INVENTION

Briefly and in general terms, a print head for ink-jet printing according to the present invention includes an orifice plate comprised of at least one metal with an intermediate layer of reinforcement material bonded or otherwise secured thereto, an ink barrier layer, and an adhesion promoter located between the intermediate layer and the barrier layer. The adhesion promoter bonds the intermediate layer to the barrier layer thereby securing the orifice plate to the barrier layer. The intermediate layer of reinforcement material preferably involves at least one silicon-containing composition. Representative compounds suitable for this purpose include but are not limited to silicon dioxide ( $\text{SiO}_2$ ), silicon nitride ( $\text{Si}_3\text{N}_4$ ), silicon carbide (SiC), and mixtures thereof. In an exemplary embodiment, the intermediate layer of reinforcement material will have a uniform thickness of about 200–10,000 angstroms.

Furthermore, the invention includes a process for making a print head for ink-jet printing comprising the steps of providing an ink-jet orifice plate comprised of at least one metal, providing an intermediate layer of reinforcement material (e.g. at least one silicon-containing composition as noted above) beneath the orifice plate, providing a layer of an adhesion promoter beneath the intermediate layer of reinforcement material, providing a barrier layer beneath the layer of adhesion promoter, and laminating the orifice plate to the barrier layer with the above-listed components thereto by applying pressure and heat.

The problem of delamination caused by aggressive inks and environmental moisture is addressed by using the intermediate layer of reinforcement material (e.g. at least one silicon-containing composition) and the selected adhesion promoter in combination between the orifice plate and the barrier layer. These materials chemically interact in a novel and effective manner which substantially improves the overall strength, durability, and structural integrity of the print head.

Other aspects and advantages of the invention will become apparent from the following detailed description, taken in conjunction with the accompanying drawing and graphs, illustrating by way of example the principles of the invention.

### BRIEF DESCRIPTION OF THE DRAWINGS

FIG. 1 is side elevational view, in cross section, of an adhesion promoter bonding an orifice plate to a barrier layer in an ink-jet print head, embodying the principles of the invention.

FIG. 2 is a plot of the work of adhesion between a barrier layer and an orifice plate having a tantalum (Ta) layer bonded thereto, using various organosilane adhesion promoters versus the number of days that a print head was soaked in ink at 60° C. depicting the improvement in the resistance to delamination as a result of organosilane adhesion promoters.

FIG. 3 is a plot of the work of adhesion between a barrier layer and an orifice plate having a chromium (Cr) layer bonded thereto, using a polyacrylic acid (PAA) adhesion promoter versus the number of days that a print head was soaked in ink at 60° C. depicting the improvement in the resistance to delamination as a result of a PAA adhesion promoter.

FIG. 4 is a plot of the push strength between a barrier layer and an orifice plate having a chromium (Cr) layer bonded thereto, using a polyacrylic acid (PAA) adhesion promoter, versus the number of days that a print head was soaked in ink at 60° C. depicting the improvement in the resistance to delamination as a result of the PAA adhesion promoter.

FIG. 5 is a plot of the push strength between a barrier layer and an orifice plate having a tantalum (Ta) layer bonded thereto, using a polyacrylic acid (PAA) adhesion promoter, versus the number of hours that a print head was soaked in ink at 60° C. depicting the improvement in the resistance to delamination as a result of the PAA adhesion promoter.

FIG. 6 is a plot of the push strength between a barrier layer and an orifice plate having a tantalum (Ta) layer bonded thereto, using a polymethylacrylic acid (PMAA) adhesion promoter, versus the number of hours that a print head was soaked in ink at 60° C. depicting the improvement in the resistance to delamination as a result of the PMAA adhesion promoter.

#### DESCRIPTION OF THE PREFERRED EMBODIMENTS

As shown in the drawings, tables and graphs, the invention is embodied in an improved print head for ink-jet printing and in a process for making such print heads.

The problem of delamination caused by aggressive inks and environmental moisture is addressed by the use of an intermediate layer of reinforcement material (discussed below) and a layer of adhesion promoter between the orifice plate and the ink barrier layer.

Referring to FIG. 1, reference numeral 12 generally indicates an ink-jet print head for ink-jet printing. The print head 12 includes an orifice plate 14 that is preferably fabricated from nickel and electroformed on a mandrel. The orifice plate 14 is about 50 microns thick. In a preferred and non-limiting embodiment, the orifice plate has a coating 16 of gold that is about 1.5 to about 3 microns thick. Other coatings 16 can be used including nickel, chromium and palladium. The orifice plate also contains a nozzle generally indicated by reference numeral 17. On the lower surface of the orifice plate 14 on the gold coating 16 is an intermediate layer 18 of reinforcement material. The intermediate layer 18 is designed to provide an enhanced degree of strength, durability, and delamination-resistance in the completed print head 12, particularly when used in cooperation with the adhesion promoters discussed below. Preferred materials used to fabricate the intermediate layer 18 of reinforcement material can be divided into two groups, both of which are related by their ability to chemically bond in an effective manner to both the selected adhesion promoter (discussed

below) and other adjacent material layers in the print head 12. The first group involves at least one oxidizable metal. In the first group, chromium, tantalum, and mixtures thereof represent preferred oxidizable metals (with tantalum providing optimum results). If an oxidizable metal is employed in connection with the intermediate layer 18, it is preferably sputtered onto the coating 16 at a representative, non-limiting thickness of about 200–1300 angstroms.

The other preferred group of materials which may be employed in connection with the intermediate layer 18 of reinforcement material involves the use of at least one silicon-containing composition. Exemplary and preferred silicon-containing compositions which are suitable for this purpose include but are not limited to silicon dioxide ( $SiO_2$ ),  
<sup>10</sup> silicon nitride ( $Si_3N_4$ ), silicon carbide (SiC), and mixtures thereof. Preferred application methods involving these materials include, for example, plasma enhanced chemical vapor deposition (also known as "PECVD") wherein the selected silicon-containing composition is optimally applied to the lower surface of the orifice plate (whether or not a gold coating 16 is employed) at an exemplary, non-limiting uniform thickness of about 200–10,000 angstroms. However, this value may be varied as needed in accordance with preliminary pilot testing. It should also be noted that  
<sup>15</sup> this group of materials (e.g. silicon-containing compositions) will work effectively with all of the various adhesion promoters discussed in detail below. Likewise, all of the assembly techniques and parameters outlined below in connection with the print head 12 are equally applicable to both groups of materials employed in connection with the intermediate layer 18 of reinforcement material.

Reference numeral 24, FIG. 1 generally indicates an ink barrier layer. The ink barrier layer 24 is fabricated from polymethylmethacrylate (PMMA) which is obtainable from  
<sup>20</sup> E. I. du Pont de Nemours and Company of Wilmington, Del.

Laminated between the intermediate layer 18 on the orifice plate and the ink barrier layer 24 is an adhesion promoter 20. The adhesion promoter 20 is formed from either organosilane, polyacrylic acid herein referred to as  
<sup>25</sup> "PAA", or polymethylacrylic acid herein referred to as "PMAA". The silanes are obtainable from the Dow Coming Corporation of Midland, Mich. and are identified in FIG. 2 and Table A by their product numbers. The PAA and the PMAA are obtainable from Polysciences, Inc. of Warrington, Pa.

Referring to FIG. 1, reference numeral 27 generally indicates a plurality of intermediate layers of various materials which are deposited on a print head substrate 29 fabricated from silicon dioxide. The barrier layer 24, the intermediate layers 27 and the substrate 29 define the firing chamber 32.

#### ORGANOSILANE ADHESION PROMOTERS

To apply the adhesion promoter 20 to the orifice plate, the orifice plate is dipped in an aqueous solution of organosilane having a concentration of between about .01% to about 1.0% in water. The preferred silane concentration is about 0.1%. After the dipping process, the orifice plate is rinsed and rotated at about 1500 rpm to remove any excess silane. The orifice plate and the layer of silane promoter are then heated for 5 minutes at 70° C. to 100° C.

A wafer, not shown, is covered with a plurality of individual print head substrates 29. Each substrate has a layer 24 of ink barrier material already cured thereon. The individual orifice plates 14 are placed on the ink barrier layers so that the orifice plates, adhesion promoter layers, and substrates

are in registration. Registration is necessary so that the architecture of the firing chambers 32 is precisely obtained.

The wafer with the orifice plates and adhesion layers in place is placed in a laminator and compressed at a pressure of about 150 psi at about 200° C. for about 10 minutes. Thereafter, the wafer is placed in an oven at 220° C. for 30 minutes. Next, each print head is sawed off the wafer and the application process is completed.

The completed print heads were tested by soaking the print heads in a solution of ink at a temperature of 60° C. for differing periods of time. Ink at an elevated temperature was used for testing in order to accelerate the delamination process. At selected times an individual print head was removed from the ink and rinsed in water. Thereafter, the print head was push tested. A force was applied perpendicularly between the orifice plate and the substrate by a mechanical tool, not shown. The force was increased until the orifice plate separated from the substrate. The amount of applied force and the movement of the tool were measured. The work of adhesion was obtained by integrating the area under the curve of applied force and the movement of the tool. The work of adhesion is measured in newton-millimeters. The push strength is the maximum force necessary to separate the orifice plate from the substrate and is measured in pounds. It is desired that the work of adhesion and the push strength be maximized.

Referring to Table A below and FIG. 2, the results of the testing are tabulated and illustrated. The following organosilanes were tested:

aminoethyl aminopropyl trimethoxysilane, Dow Coming Z-6020

3-chloropropyl trimethoxysilane, Dow Coming Z-6026

glycidoxypropyl trimethoxysilane, Dow Coming Z-6040

gamma-aminopropyl triethoxysilane, Dow Coming Z-6011

methacryloxypropyl trimethoxysilane, Dow Coming Z-6030.

The controls were orifice plates without adhesion promoters and, in particular, orifice plates with either an intermediate layer 18 of Palladium (Pd) or an intermediate layer 18 of Tantalum (Ta).

TABLE A

| Work of Adhesion (newton-mm) of Tantalum with Organosilane Adhesion Promoters |                          |                    |       |       |       |       |        |
|-------------------------------------------------------------------------------|--------------------------|--------------------|-------|-------|-------|-------|--------|
| Number                                                                        | Coating on Orifice Plate | Adhesion Promoters | Day 0 | Day 1 | Day 3 | Day 6 | Day 14 |
| 1                                                                             | Ta                       | 6020               | 18.31 | 8.70  | 7.16  | 6.85  | 6.03   |
| 2                                                                             | Ta                       | 6030               | 18.28 | 8.65  | 7.08  | 5.18  | 4.97   |
| 3                                                                             | Ta                       | 6011               | 15.46 | 8.58  | 5.83  | 6.01  | 5.91   |
| 4                                                                             | Ta                       | 6040               | 17.35 | 8.43  | 6.52  | 5.60  | 5.56   |
| control                                                                       | Ta                       | none               | 17.53 | 7.14  | 1.17  | 0.50  | 0.41   |
|                                                                               |                          |                    |       |       |       |       | —      |

It should be appreciated from FIG. 2 that after about three days of soaking in ink at 60° C., the orifice plates without an adhesion promoter had essentially fallen off of the substrate. These were the orifice plates with just layers of Palladium (pd) and Tantalum (Ta) only.

#### POLYACRYLIC ACID (PAA) AND POLYMETHYLACRYLIC ACID (PMAA) ADHESION PROMOTERS

The PAA is applied to the orifice plates by first dipping the orifice plates in a 1% solution of PAA for 3 minutes and then

drying the orifice plates in an oven at 150° C. for 5 minutes. The orifice plates are thereafter washed in deionized water at 50° C. for 30 minutes. During the washing process the orifice plates are agitated. Next, the orifice plates are air dried and laminated to the print head substrate as described above.

For PAA a molecular weight of between 90,000 and 250,000 daltons is used and a molecular weight of about 100,000 to 200,000 daltons is preferred.

In addition, a thickness of less than 5 monolayers of PAA on the orifice plate is preferred. This thin layer is obtained by controlling the concentration of PAA solution and the water rinse time as described above. A concentration of PAA of between 0.05% and 10% is used and a concentration of 1.0% in water is preferred.

FIGS. 3 and 4 and Tables B and C below illustrate Cr with PAA and also the correspondence of the work of adhesion with push strength for the same materials over the same periods of time.

TABLE B

| Work of Adhesion (newton-millimeters) of Chromium with and without Polyacrylic Acid (PAA) Adhesion Promoters |                          |       |       |       |       |        |
|--------------------------------------------------------------------------------------------------------------|--------------------------|-------|-------|-------|-------|--------|
| Number                                                                                                       | Coating on Orifice Plate | Day 0 | Day 1 | Day 3 | Day 6 | Day 16 |
| 1                                                                                                            | Cr                       | 11.91 | 6.34  | 3.7   | 1.55  | 1.39   |
| 2                                                                                                            | Cr + PAA                 | 16.9  | 9.25  | 8.91  | 3.34  | 4.7    |

TABLE C

| Push Strength (lbs.) Of Chromium with and without Polyacrylic Acid (PAA) Adhesion Promoters |                          |       |       |       |       |        |
|---------------------------------------------------------------------------------------------|--------------------------|-------|-------|-------|-------|--------|
| Numbers                                                                                     | Coating on Orifice Plate | Day 0 | Day 1 | Day 3 | Day 6 | Day 16 |
| 1                                                                                           | Cr                       | 9.52  | 4.82  | 2.13  | 1.06  | 0.76   |
| 2                                                                                           | Cr + PAA                 | 10.3  | 6.6   | 4.72  | 2.43  | 2.2    |

50 The ink used in Table E and FIG. 6 was different from the ink used in the other tables and figures. This other ink was used in all tests except Table E and FIG. 6

TABLE D

| Push Strength (lbs.) Of Tantalum with and without Polyacrylic Acid (PAA) Adhesion Promoters |                          |          |          |           |
|---------------------------------------------------------------------------------------------|--------------------------|----------|----------|-----------|
| Number                                                                                      | Coating on Orifice Plate | Hours 71 | Hours 23 | Hours 172 |
| 1                                                                                           | Ta                       | 2.1      | 1.8      | 1.6       |
| 2                                                                                           | Ta + PAA                 | 8.5      | 6.4      | 5.2       |

65 For the PMAA adhesion promoter, Table E, the orifice plates are prepared and the PMAA is applied in the same manner as described above.

TABLE E

| Push Strength (lbs.) Of Palladium and Polymethylacrylic Acid (PMAA) Adhesion Promotor on Tantalum |                                |      |     |     |     |     |      |      |      |    |
|---------------------------------------------------------------------------------------------------|--------------------------------|------|-----|-----|-----|-----|------|------|------|----|
| No.                                                                                               | Coating of<br>Orifice<br>Plate | Hrs. |     |     |     |     |      |      |      |    |
|                                                                                                   |                                | 52   | 169 | 336 | 405 | 504 | 692  | 836  | 1005 | 10 |
| 1                                                                                                 | Pd                             | 7.8  | 6.1 | 2.5 | 1.4 | 0.4 | 0.22 | 0.21 | 0.21 | 5  |
| 2                                                                                                 | PMAA<br>+ Ta                   |      | 9.3 | 7.7 |     | 7.7 | 7.5  | 6.5  | 7.0  | 10 |

Table E compares ink soak testing of Palladium only orifice plates to PMAA on tantalum sputtered on Palladium coated orifice plates. 15

Although specific embodiments and processes of the invention have been described and illustrated, the invention is not to be limited to the specific forms or arrangement of parts so described and illustrated. The invention is limited only by the claims. 20

We claim:

1. A print head for ink-jet printing, comprising:  
an orifice plate comprised of at least one metal;  
an intermediate layer of reinforcement material bonded to  
said orifice plate, said intermediate layer being com-  
prised of at least one silicon-containing composition  
selected from the group consisting of silicon dioxide,  
silicon nitride, silicon carbide, and mixtures thereof;  
an ink barrier layer comprised of an organic polymer  
composition; and  
an organic adhesion promoter positioned between said  
intermediate layer and said ink barrier layer, said  
organic adhesion promoter bonding said intermediate  
layer to said ink barrier layer in order to prevent  
detachment of said orifice plate from said print head,  
said organic adhesion promoter being selected from the  
group consisting of polyacrylic acid, polymethylacrylic  
acid, an organosilane composition, and mixtures  
thereof. 25
2. The print head of claim 1 wherein said polyacrylic acid  
has a molecular weight of about 90,000-250,000 daltons.
3. The print head of claim 1 wherein said organosilane  
composition is selected from the group consisting of ami-  
noethyl aminopropyl trimethoxysilane, 3-chloropropyl  
trimethoxysilane, glycidoxypropyl trimethoxysilane,  
gamma-aminopropyl triethoxysilane, methacryloxypropyl  
trimethoxysilane, and mixtures thereof. 45
4. The print head of claim 1 wherein said intermediate  
layer has a thickness of about 200-10,000 angstroms. 50
5. A print head for ink-jet printing, comprising:  
an orifice plate comprised of at least one metal;  
an intermediate layer of reinforcement material bonded to  
said orifice plate, said intermediate layer being com-  
prised of at least one silicon-containing composition;  
an ink barrier layer comprised of an organic polymer  
composition; and  
an organic adhesion promoter positioned between said  
intermediate layer and said ink barrier layer, said  
organic adhesion promoter bonding said intermediate  
layer to said ink barrier layer in order to prevent  
detachment of said orifice plate from said print head,  
said organic adhesion promoter being selected from the  
group consisting of polyacrylic acid, polymethylacrylic  
acid, an organosilane composition, and mixtures  
thereof. 60

## 8

layer to said ink barrier layer in order to prevent  
detachment of said orifice plate from said print head,  
said organic adhesion promoter being selected from the  
group consisting of polyacrylic acid, polymethylacrylic  
acid, an organosilane composition, and mixtures  
thereof.

6. A method for producing an ink-jet print head comprising:

providing an orifice plate comprised of at least one metal,  
said orifice plate further comprising an intermediate  
layer of reinforcement material bonded thereto, said  
intermediate layer being comprised of at least one  
silicon-containing composition selected from the group  
consisting of silicon dioxide, silicon nitride, silicon  
carbide, and mixtures thereof;

providing an ink barrier layer comprised of an organic  
polymer composition; and

adhering said orifice plate to said ink barrier layer using  
an organic adhesion promoter positioned between said  
intermediate layer on said orifice plate and said ink  
barrier layer, said organic adhesion promoter bonding  
said intermediate layer to said ink barrier layer in order  
to prevent detachment of said orifice plate from said  
print head, said organic adhesion promoter being  
selected from the group consisting of polyacrylic acid,  
polymethylacrylic acid, an organosilane composition,  
and mixtures thereof.

7. The method of claim 6 wherein said adhering of said  
orifice plate to said ink barrier layer comprises compressing  
said orifice plate and said ink barrier layer together with said  
organic adhesion promoter therebetween in an amount suf-  
ficient to secure said orifice plate to said ink barrier layer. 30

8. The method of claim 6 wherein said organosilane  
composition is selected from the group consisting of ami-  
noethyl aminopropyl trimethoxysilane, 3-chloropropyl  
trimethoxysilane, glycidoxypropyl trimethoxysilane,  
gamma-aminopropyl triethoxysilane, methacryloxypropyl  
trimethoxysilane, and mixtures thereof. 35

9. The method of claim 6 wherein said intermediate layer  
has a thickness of about 200-10,000 angstroms.

10. A method for producing an ink-jet print head comprising:

providing an orifice plate comprised of at least one metal,  
said orifice plate further comprising an intermediate  
layer of reinforcement material bonded thereto, said  
intermediate layer being comprised of at least one  
silicon-containing composition;

providing an ink barrier layer comprised of an organic  
polymer composition; and

adhering said orifice plate to said ink barrier layer using  
an organic adhesion promoter positioned between said  
intermediate layer on said orifice plate and said ink  
barrier layer, said organic adhesion promoter bonding  
said intermediate layer to said ink barrier layer in order  
to prevent detachment of said orifice plate from said  
print head, said organic adhesion promoter being  
selected from the group consisting of polyacrylic acid,  
polymethylacrylic acid, an organosilane composition,  
and mixtures thereof.

\* \* \* \* \*